

Feb. 20, 1951

C. L. R. DE WET  
SANITARY NAPKIN

2,542,909

Filed Aug. 23, 1949

Fig. 1



Fig. 2



Inventor:  
Charl Louis Roux de Wet  
By: Soans, Pond, & Anderson  
Atty's.

## UNITED STATES PATENT OFFICE

2,542,909

## SANITARY NAPKIN

Charl Louis Roux de Wet, Neenah, Wis., assignor  
to International Cellucotton Products Company,  
Chicago, Ill., a corporation of Delaware

Application August 23, 1949, Serial No. 111,953

6 Claims. (Cl. 167—84)

1

The present invention relates to catamenial bandages or sanitary napkins and is of particular value for mitigating odors produced by the body excretions absorbed by such bandages, whether such odors are initially present in the secretions or are subsequently developed.

Various attempts have been made to mitigate the odors which sometimes develop incident to the use of catamenial bandages. Reference may be had to the prior U. S. patents to Cline, No. 2,024,145, issued December 17, 1935, and to Williams, No. 2,067,961, issued January 19, 1937. Also, various types of deodorizing agents have been employed for the purpose indicated, for example, metallic peroxides such as zinc peroxide, the use of which is suggested in the patent to Melton, No. 2,144,632. However, the efficiency of such known methods and materials has not been entirely satisfactory in certain cases.

One of the most effective of the known methods of deodorizing sanitary napkins includes the incorporation of zinc peroxide into the napkin. The deodorizing effect of zinc peroxide appears to be due, in part, to the liberation of oxygen by reason of the chemical reaction which takes place between the zinc peroxide and the liquid body excretion. Notwithstanding the widespread use of zinc peroxide as a deodorant for the purpose, its use under certain conditions causes the development of an odor which is different than the original odor of the exudate but which is objectionable to some persons. Furthermore, relatively large amounts of zinc peroxide are required to produce a noticeable reduction in odor, and the inclusion of large amounts of the zinc peroxide, a substantially insoluble compound, reduces the absorptivity of the pad and thereby impairs its efficiency.

I have found that, although the liberation of oxygen may be of considerable value in removing odors and in preventing odors from developing, the efficiency, i. e. the percentage of cases where the development of odors is prevented or mitigated, may be greatly increased by the addition to a napkin of one or more quaternary ammonium compounds in combination with a relatively small amount of zinc peroxide. The quaternary ammonium compounds have many important properties which enhance their effectiveness in a sanitary napkin, e. g. they are colorless and odorless, and in the concentrations employed are non-toxic and non-irritating. Moreover, these quaternary compounds serve to soften the fibers of the napkin and are not readily leached away from the zone in which they are needed during

use. Certain of the quaternary ammonium compounds by themselves may be employed in combination with a cellulosic carrier to effect deodorization of liquid body excretions as described in my co-pending application Serial No. 105,901 which was filed on July 20, 1949.

In the event that certain of the quaternary ammonium compounds are employed by themselves in mitigating odors from body excretions, there is a reaction between the odorless quaternary ammonium compound and the body excretion which produces, under some conditions, an aromatic odor which has been found objectionable by some persons. When the zinc peroxide and the quaternary ammonium compound are introduced into the napkin together, the combined action of the two materials is effective to eliminate substantially all traces of odor, and this deodorizing action is effective over a prolonged period of time.

Among the quaternary ammonium compounds which have been successfully used in combination with zinc peroxide and by the use of which extremely high deodorizing efficiency is obtained are the following:

1. Alkyl (8 to 18 carbon atoms) dimethyl benzyl ammonium chloride;
2. Di-isobutyl cresoxy ethoxy ethyl dimethyl benzyl ammonium chloride, which compound may be prepared by following procedures similar to those disclosed in Bock Patents Nos. 2,297,531, 2,282,702, 2,276,149 and 2,204,653, and in Bruson Patents Nos. 2,170,111, 2,225,250, and 2,132,674;
3. N (higher acyl esters of colamino formyl) (methyl) pyridinium chloride whose structural formula is



where  $n$  is at least 2;

4. Di-isobutyl phenoxy-ethoxy-ethyl di-methyl benzyl ammonium chloride, which compound may be prepared in a manner similar to that set forth in connection with compound 2 above;
5. Lauryl pyridinium chloride.

My investigations have shown that a sanitary napkin or catamenial bandage should, for proper deodorization, have incorporated therein at least 15 mg. (milligrams) of commercial zinc peroxide (50 per cent active zinc peroxide and 50 per cent zinc oxide) and from 1.5 to 30 mg. of the quaternary ammonium compound. This material de-

sirably should be incorporated into an active portion of the napkin, i. e. a portion of the napkin through which the excretion will pass. Extensive tests have shown that a napkin, for example, containing 20 mg. commercial zinc peroxide and 6 mg. of a quaternary ammonium compound (0.026 gram of the mixture) is as effective in mitigating odors as from about 1 to 5 grams of commercial zinc peroxide alone. Thus, it will be seen that on a comparative weight basis, my improved deodorant is from about 40 to 200 times as effective as zinc peroxide. Further, a sanitary napkin which contains my improved composition completely deodorizes the exudate, and there are no new odors formed in the sanitary napkin as a result of the deodorization of the excretions. In other words, the napkin is odorless before, during, and after use.

The preferred proportions of zinc peroxide and the quaternary ammonium compound per napkin are from about 20-40 mg. of commercial zinc peroxide and to from about 6 to 15 mg. of the quaternary ammonium compounds. All of the quaternary ammonium compounds will produce a marked deodorizing effect when combined with zinc peroxide, however, those compounds which have been set forth above have produced extremely effective deodorization efficiencies.

#### Specific Example

In the drawing accompanying this application, Fig. 1 is a diagrammatic view showing the equipment and process used for producing a deodorizing strip for incorporation in a sanitary napkin, and constructed in accordance with my invention; and

Fig. 2 is a perspective view showing a catamenial bandage equipped with one of my improved deodorizing strips.

In the drawing, Fig. 1, a supply roll 10 of suitable permeable material is shown in position to be impregnated with a deodorant composition in accordance with the invention. In the present instance the permeable material is paper wadding or tissue of a type similar to that which is used for facial tissues or for the plies of absorbent wadding. The sheet employed has a dry weight of about 8 lbs. to the ream of 3,000 square feet, with a creping ratio of between 1.5 and 2.0, although lighter or heavier sheets with different ratios of creping, may be employed, if needed, to suit other conditions.

The web of untreated creped wadding passes over idler rolls 12 and 13 to the nip of a pair of coating rolls comprising an applicator roll 14, preferably provided with a soft rubber exterior, and a drying and creping roll 15. The applicator roll 14 is positioned so its lower surface is wetted by the liquid 16 contained in a suitable trough 17. The liquid is rapidly circulated through the trough 17 by means of a pump 18 and suitable piping connections 19 and 20. The supply of treating liquid 16 in the trough 17 is maintained by feeding into the trough additional liquid through a liquid supply line 21.

Said liquid 16 comprises a liquid dispersion of a suitable adhesive and contains in suspension or solution the active ingredients of the deodorizing material. The adhesive is a water dispersion of boiled or gelatinized starch but other adhesives may be used. A relatively small amount of adhesive is required. Good results have been obtained by using a good grade of cooked, soluble starch in an amount representing about 9% of

the dry weight of the total solids used in the formula.

To insure a proper dispersion or suspension it may be advisable to use a small percentage of a dispersing agent. In such cases, I have successfully used .4% (based upon the dry weight of the total solids) of sodium hexametaphosphate. A typical formula for the slurry which contains the deodorizing substances is the following:

|    |                                                                                         |       |      |
|----|-----------------------------------------------------------------------------------------|-------|------|
| 10 | Commercial zinc peroxide (containing 50% of the pure chemical and 50% of zinc oxide)    | grams | 400  |
| 15 | Adsorptive paper-coating clay                                                           | do    | 800  |
| 20 | Boric acid                                                                              | do    | 120  |
| 25 | Starch (adhesive)                                                                       | do    | 144  |
| 30 | Sodium hexametaphosphate (dispersing agent)                                             | grams | 6    |
| 35 | Di'-isobutyl cresoxy - ethoxy - ethyl di-methyl benzyl ammonium chloride (25% solution) | cc    | 480  |
| 40 | Water                                                                                   | cc    | 4020 |

Thus, it may be seen that the slurry contains, on the dry basis, about 25 per cent of commercial zinc peroxide, about 8 per cent of boric acid; and about 8 per cent of the pure quaternary ammonium compound. This means that in the slurry there are about 25 parts by weight of commercial zinc peroxide to about 8 parts by weight of boric acid and about 8 parts by weight of the pure quaternary ammonium compound.

The use of boric acid appears to be of advantage in increasing the acidity of the body excretion to a pH of about 6.5 to 7.5. This reduces the tendency of the excretion to irritate the skin. Instead of boric acid, I may use other weak acids, such as citric or tartaric, such acidic salts as mono-ammonium phosphate; ammonium sulphate or zinc sulphate or salts such as ammonium di-basic phosphate which becomes acidic upon heating. According to my present information, it is not advisable to use relatively stronger or more reactive acids which, when incorporated with the other ingredients, appear to produce premature or undesirable reactions.

The clay acts as an adsorbent. The purpose of the other ingredients has already been described. In some cases, the adhesive, clay, and weak acid may be omitted.

Sufficient pressure is applied to the rubber faced applicator roll 14, and the consistency or amount of water in the liquid dispersion is suitably adjusted, so that the proper amount of material is applied to the web 11 when it passes through the nip of the coating rolls 14 and 15. For the purpose indicated, the slurry may conveniently have a consistency of about 25 per cent solids, and the pressure between the rolls is adjusted so that after the strip is dried, the total added solids content will be about 50% of the weight of fiber in the sheet.

Sufficient heat is applied to the interior of the creping roll 15 to drive off a substantial percentage of the water of the dispersion. Enough water is driven off to bring the sheet into proper condition of dryness to be removed and creped by the usual creping doctor 22. From the creping doctor 22, the treated sheet passes under an idler roll 23 and around a set of driers, for example three driers 24, 25 and 26, which complete the drying of the sheet to a moisture content of normal paper dryness, i. e. containing about 5% of moisture. If the sheet is of substantial width, it may then be slit into strips of the proper width by means of a slitting mechanism indicated at

27 from which it passes to a re-winding arrangement indicated generally at 28.

When the strip is to be used for deodorizing sanitary napkins of the usual construction, it will preferably have been cut to a width slightly less than the width of the fibrous, absorbent, liquid permeable element of the sanitary napkin, and such strip is made up in lengths long enough to cover an area equal to the zone of contact between the napkin and the person of the wearer. For example, a strip may conveniently be about 5 inches long and slightly less than 3 inches wide. If a single strip is to be employed in a sanitary napkin, the operation is adjusted so that the strip will contain say 20 mg. of commercial zinc peroxide and 6 mg. of di-isobutyl-cresoxy ethoxy dimethyl benzyl ammonium chloride.

The deodorizing strip 29 is incorporated to the absorbent element 30 of the napkin which is equipped with the usual gauze wrapper 31 the folds of which are shown folded back to expose the interior construction. Said strip may be employed on either side of the element 30, as shown at 29 or 29', or it may be incorporated in the center of the pad as shown at 29".

Tests which have been carried out to ascertain the deodorizing effect of sanitary napkins which have been made in accordance with the foregoing specific example have shown that the deodorizing effect in the napkin is equivalent to the deodorizing effect obtained when about 2½ grams of commercial zinc peroxide is incorporated in a napkin. Thus, it will be seen that on a weight basis, the deodorizing composition in accordance with the specific example is 100 times as effective as an equivalent weight of zinc peroxide. The element containing the combination of the zinc peroxide and the quaternary ammonium compound is soft and pliable and has substantially all of its original absorptivity.

The slurry employed in applying the mixture of zinc peroxide and quaternary ammonium compound to the deodorizing strip has been found to be stable in water so that there is little danger that the activity of the mixture will be reduced by circulating the slurry through the trough 17.

This application is a continuation-in-part of my prior application Serial No. 630,828 which was filed on November 26, 1945, and is now abandoned, and which is assigned to the assignee of this invention.

Various features of the invention which are believed to be new are set forth in the appended claims.

I claim:

1. A sanitary napkin which includes a fibrous, liquid permeable, absorbent element and a deodorant distributed throughout the active portion thereof, the said deodorant comprising from

about 1.5 to 30.0 milligrams of a quaternary ammonium compound and over about 15 milligrams of commercial zinc peroxide.

5 2. A sanitary napkin which includes a fibrous, liquid permeable, absorbent element and a deodorant distributed throughout the active portion thereof, the said deodorant comprising from about 1.5 to 30.0 milligrams of a quaternary ammonium compound and from about 20 to 40 milligrams of commercial zinc peroxide.

10 3. A sanitary napkin which includes a fibrous, liquid permeable, absorbent element and a deodorant distributed throughout the active portion thereof, the said deodorant comprising from about 6 to 15 milligrams of a quaternary ammonium compound and from about 20 to 40 milligrams of commercial zinc peroxide.

15 4. A sanitary napkin which includes a fibrous, liquid permeable, absorbent element and a deodorant distributed through the active portion thereof, the said deodorant comprising from 1.5 to 30.0 milligrams of di-isobutyl cresoxy ethoxy ethyl dimethyl benzyl ammonium chloride and from about 20 to 40 milligrams of commercial zinc peroxide.

20 5. A sanitary napkin which includes a fibrous, liquid permeable, absorbent element and a deodorant distributed throughout the active portion thereof, the said deodorant comprising from about 1.5 to 30.0 milligrams of di-isobutyl phenoxy ethoxy ethyl dimethyl benzyl ammonium chloride and from about 20 to 40 milligrams of commercial zinc peroxide.

25 6. A sanitary napkin which includes a fibrous, liquid permeable, absorbent element and a deodorant distributed throughout the active portion thereof, the said deodorant comprising from about 1.5 to 30.0 milligrams of alkyl dimethyl benzyl ammonium chloride, said alkyl group containing from 8 to 18 carbon atoms and from about 20 to 40 milligrams of commercial zinc peroxide.

CHARL LOUIS ROUX DE WET.

#### REFERENCES CITED

The following references are of record in the file of this patent:

#### UNITED STATES PATENTS

| Number    | Name           | Date           |
|-----------|----------------|----------------|
| 1,950,286 | Barkow         | Mar. 6, 1934   |
| 1,953,526 | Ainsley et al. | Apr. 3, 1934   |
| 2,024,145 | Cline          | Dec. 17, 1935  |
| 2,131,235 | Randall et al. | Sept. 27, 1938 |

#### OTHER REFERENCES

Annals of Surgery, Oct. 1943, page 744.  
Drug and Cosmetic Industry, Nov. 1943, page